

March 17, 1925.

1,530,281

J. L. MURRIE

## MANUFACTURE OF GAS

Filed July 26, 1923



INVENTOR  
John Lester Murrie  
BY Edward R. Knowles.  
ATTORNEY

Patented Mar. 17, 1925.

## UNITED STATES PATENT OFFICE.

JOHN LESTER MURRIE, OF YONKERS, NEW YORK.

## MANUFACTURE OF GAS.

Application filed July 26, 1923. Serial No. 654,042.

*To all whom it may concern:*

Be it known that I, JOHN LESTER MURRIE, a citizen of the United States, residing at Yonkers, in the county of Westchester and State of New York, have invented certain new and useful Improvements in the Manufacture of Gas, of which the following is a specification.

My invention relates to the formation of gas suitable for light, heat and power purposes directly from coal by its combination with superheated steam at a high temperature.

I have found that when coal in a finely pulverized condition is mixed with superheated steam in a suitably proportioned coil and submitted to a high temperature the volatile hydrocarbons in the coal are set free and disassociated by the heat into their hydrogen and carbon components. At the same time the steam is disassociated into its hydrogen and oxygen components. New combinations of the free hydrogen, carbon and oxygen units take place, depending upon the proportions of finely pulverized coal and steam used and the temperature to which the mixture is submitted, thus forming fixed gases of a high B. t. u. value, which can be used, after purification by washing, as a fuel gas and possibly as an illuminating gas.

If finely powdered coal and superheated steam are mixed in a confined space and subjected to a high temperature, the action is violent and explosive in character, being substantially instantaneous, but by making the space in which the action takes place of a gradually expanding form, the action takes place more slowly and progressively.

My invention relates to a process for manufacturing gas as indicated above, and also to a suitable apparatus for carrying out the process in an advantageous manner.

Other features of novelty will be apparent from the following detailed description and the appended claims.

In the drawings:

Figure 1 is a longitudinal vertical section of one form of apparatus used in connection with a steam boiler to utilize the high furnace heat of the same.

Figure 2 is a longitudinal section of one form of device for feeding pulverized coal and supplying superheated steam thereto.

Figure 2<sup>a</sup> is a longitudinal section of another form of feeding apparatus.

Figure 3 is a vertical section of a form of furnace for heating the gasifying coil, utilizing gas or oil as a fuel.

As illustrated in Figure 1, A. is a typical steam boiler of the horizontal water tube type in which are employed water tubes 1, a water and steam drum 2, combustion chamber 3, a boiler setting 4, a superheater 5 and smoke flue 5<sup>a</sup>.

In the form shown, the boiler is fired with pulverized coal by means of the apparatus C in which a pulverizer 7 is driven by an electric motor 11. The coal is fed to the pulverizer 7 from a hopper 10 which in turn receives the coal from a bunker or other container 12 through a pipe 13 provided with a valve or cut-off 14 for controlling the supply of coal. The pulverized coal is delivered from the pulverizer 7 to the combustion chamber through the flue 8 and tuyère 9.

The combustion of the pulverized coal in the combustion chamber generates highly heated gases which generate steam in the boiler. Of course, as hereinafter set forth, any other form of heating the boiler or other chamber may be employed.

In the combustion chamber is located a pipe coil 6 which is preferably made tapering as shown, increasing gradually in area from its inlet end to a much larger area at its outlet end, as shown in Figures 1 and 3. The shape, size and arrangement of the coil may be varied as desired, but it should always increase in area to obtain the best results and enable the combination to take place more or less gradually and uniformly.

The inlet end of the coil 6 extends outside of the boiler setting and is connected to the pulverized coal and steam feeding mechanism D of Figures 1 and 2 or D' of Figure 2<sup>a</sup>.

This feeding mechanism may be of various forms, two of which are illustrated. As shown in Figure 2 it consists of a cylinder 18 in which is enclosed a worm 19 which fits the interior of the cylinder closely and which can be rotated at any desired speed by means of the variable speed motor which is connected to the shaft 41 of the worm 19. From the main pulverized coal feed 8 a branch pipe 15 diverts a portion of the pulverized coal to the hopper 17 from which it is fed by a pipe 40<sup>a</sup> to the cylinder 18. The relative amounts of coal which pass to the combustion chamber and to the hopper 17 are varied by an adjustable damper 51 lo-

cated at the juncture of the pipes 8 and 15. The force of the pulverizer is sufficient to deliver the pulverized coal through the conduit 15 as well as through the pipe 8 to the combustion chamber. The flow of the coal through the pipe 15 may further be controlled by a valve 31.

The outlet 40 for the coal from the cylinder 18 is connected to the steam jet box 20 which in turn is connected to the inlet end of the coil 6. A steam pipe 21 for delivering a jet of superheated steam is placed axially in the steam jet box 20, and is connected to the superheater 5 by pipes 22, 24 and 23, 15 which are controlled by valves 26, 27, 28, 29 and 30. A pipe 23<sup>a</sup> from the steam space 23<sup>b</sup> in the water and steam drum 2 communicates with the superheater.

The outlet end of coil 6 is connected by pipe 32 controlled by valve 33 to a discharge pipe 34 located within the water 37 in a tank 36 of a gas holder B which also comprises a bell 35 having its lower end submerged in the water 37. A gas outlet pipe 38 controlled by valve 39 connects the interior of the bell to a desired outside point.

The process is carried out in the above described apparatus as follows:—

The finely pulverized coal is fed from the pulverizer into the boiler furnace 3 where complete combustion takes place and the furnace is heated to a high temperature. The expanding coil 6 is thereby heated to approximately the same temperature. When the coil 6 is properly heated superheated steam is admitted in a controlled amount, through jet 21 and at the same time, by the revolution of the screw 19 the desired amount of pulverized coal is fed from hopper 17 through pipe 40<sup>a</sup>, screw 19 and pipe 40 into the space in tube 20 surrounding the steam jet 21. The suction created by the jet of steam issuing from the jet nozzle at high velocity draws with it the pulverized coal which is instantaneously mixed with the steam, the mixture passing into expanding coil 6 where, owing to the high temperature to which it is submitted, the particles of the pulverized coal are split up into their component units of carbon, hydrogen, and oxygen, and the steam is also disassociated into its component units of hydrogen and oxygen. As these free intermingled units of carbon, hydrogen and oxygen pass through the expanding coil 6, they recombine and form a gas of high B. t. u. value. Due to the increasing volume of the coil 6 this action takes place gradually and the gas becomes a saturated fixed gas which passes through the pipes 32 and 34 and passes up through the water in tank 36.

No coking action takes place and there is no coke residue. The small amount of ash that is formed passes through with the gas and is washed out by the water in the gas

tank or by any other suitable means. The washed gas may be drawn off from the bell 35 for any desired purpose.

The process is continuous and may be carried out so long as the pulverized coal and the superheated steam are fed in the right proportions into coil 6. This is regulated by the steam control valve 30, the valves 31 and 51, and the speed of the feed screw 19.

One important features of this process is the employment of an expanding coil whereby the gas formation is permitted to take place gradually and progressively and not explosively as would be the case if the pulverized coal and superheated steam were allowed to mix in a small confined space at high temperature.

In Figure 3 a furnace E has walls 41 and 42 provided with an expanding coil 6 and pulverized coal injecting apparatus similar to that of Figures 1 and 2. This furnace is fired by a gas or oil burner 48, the gas or oil being fed through pipe 44 controlled by a valve 46 and the air being fed through pipe 45 controlled by valve 47. The heated gases from the furnace pass through outlet flue 42 provided with a control damper 43. The action of this furnace is similar to that already described.

A modified form of feeding apparatus is disclosed in Figure 2<sup>a</sup> and comprises a drum 18<sup>a</sup> interposed between the hopper 17 and the outlet pipe 40. In this drum there rotates a member 4<sup>a</sup> having arms 19<sup>a</sup> the ends of which clear the walls of the drum 18<sup>a</sup> forming pockets 19<sup>b</sup> which carry the coal from the hopper 17 to the pipe 40. In other respects the mechanism resembles that already described, and it is obvious that the feeding mechanism D' may be used with the furnace shown in Figure 1 or with that shown in Figure 3. For that matter, other forms of feeding mechanisms may be used with other forms of furnaces, so long as certain essential features are present.

It will be noted that the process is carried out with the practical exclusion of air or any oxygen except that obtained by the decomposition of the constituents. The feeding arrangement shown in Figure 2<sup>a</sup> particularly substantially prevents the entrance of air from the outside, and that employed in Figures 1 and 2 will also substantially prevent any air from entering the coil when in use. This is an important feature of the process which operates with greater efficiency if the supply of oxygen is limited to that resulting from the breaking down of the coal and the steam.

Obviously certain modifications may be made without departing from the spirit of the invention, and the process itself is independent of any specific apparatus. The invention is therefore to be regarded as lim-

ited only by the scope of the appended claims.

I claim as my invention:

1. The process of forming a gas of high B. t. u. value direct from solid carbonaceous material which comprises finely pulverizing the material, mixing it with superheated steam, and exposing the mixture to 15 a high temperature in a gradually expanding coil with the substantial exclusion of air or extraneous oxygen.
- 5 B. t. u. value direct from solid carbonaceous material which comprises finely pulverizing the material, mixing it with superheated steam, and exposing the mixture to a high temperature in a coil whose volume 10 gradually increases from end to end.
- 10 2. The process of forming a gas of high

B. t. u. value direct from solid carbonaceous material which comprises finely pulverizing the material, mixing it with superheated steam, and exposing the mixture to 15 a high temperature in a gradually expanding coil with the substantial exclusion of air or extraneous oxygen.

In testimony whereof I affix my signature.

JOHN LESTER MURRIE.